

Oct. 18, 1938.

T. S. HODGINS

2,133,894

PROCESS FOR IMPROVING DRYING PROPERTIES OF OILS

Filed Feb. 26, 1937

8 Sheets-Sheet 1

Fig. 1.



Fig. 2.



Inventor

T. S. Hodgins,

Attorneys

By Munson H. Lane,

Oct. 18, 1938.

T. S. HODGINS

2,133,894

PROCESS FOR IMPROVING DRYING PROPERTIES OF OILS

Filed Feb. 26, 1937

8 Sheets-Sheet 2

Fig. 3.



T. S. Hodgins

By Munson H. Lane,

Attorney

Oct. 18, 1938.

T. S. HODGINS

2,133,894

PROCESS FOR IMPROVING DRYING PROPERTIES OF OILS

Filed Feb. 26, 1937

8 Sheets-Sheet 3

Fig. 4.



By Munson H. Lane,

Attorney

Oct. 18, 1938.

T. S. HODGINS

2,133,894

PROCESS FOR IMPROVING DRYING PROPERTIES OF OILS

Filed Feb. 26, 1937

8 Sheets-Sheet 4

Fig. 5.

ALKALI-PERMANGANATE SAMPLES



Inventor

*T. S. Hodgins,*

By *Munson H. Lane,*

Attorney

Oct. 18, 1938.

T. S. HODGINS

2,133,894

PROCESS FOR IMPROVING DRYING PROPERTIES OF OILS

Filed Feb. 26, 1937

8 Sheets-Sheet 5

Fig. 6.



Inventor

*T.S. Hodgins*

By *Munson H. Lane*,

Attorney

Oct. 18, 1938.

T. S. HODGINS

2,133,894

PROCESS FOR IMPROVING DRYING PROPERTIES OF OILS

Filed Feb. 26, 1937

8 Sheets-Sheet 6

Fig. 7.



By Munson H. Lane,

Attorneys

Oct. 18, 1938.

T. S. HODGINS

2,133,894

PROCESS FOR IMPROVING DRYING PROPERTIES OF OILS

Filed Feb. 26, 1937

8 Sheets-Sheet 7

*Fig. 8*

HNO<sub>3</sub> TREATED SAMPLES



J. Inventor

*T. S. Hodgins,*

*Munson A. Lane,*

Attorney

Oct. 18, 1938.

T. S. HODGINS

2,133,894

PROCESS FOR IMPROVING DRYING PROPERTIES OF OILS

Filed Feb. 26, 1937

8 Sheets-Sheet 8

Fig. 9.



Inventor

T. S. Hodgins,  
By Munson H. Lane, Attorney

## UNITED STATES PATENT OFFICE

2,133,894

PROCESS FOR IMPROVING DRYING  
PROPERTIES OF OILSTheodore S. Hodgins, Detroit, Mich., assignor to  
Helmut Reichhold, doing business as Reich-  
hold Chemicals, Detroit, Mich.

Application February 26, 1937, Serial No. 127,971

3 Claims. (Cl. 260—423)

This invention relates to a process for improving the drying properties of raw oils by removing anti-oxidants therefrom, so as to render the oils more suitable for use in the paint and kindred industries.

I am aware that previous attempts have been made to improve the drying properties of oils by partially oxidizing the same, particularly by passing air or other oxidizing gas through the body of the oil. My invention is not concerned with this type of oxidation. In such prior processes the oxidation has taken place within the oil itself whereas according to my process only the anti-oxidants are eliminated, the oil being unoxidized. Also in such previous treatments temperatures above room temperature have been considered necessary whereas my process may be carried on to best advantage at substantially room temperature.

It has also been proposed to treat various oils with chemical reagents such as acids, alkalies and salts for the purpose of improving their qualities, as for example for removing odors, or for bleaching the same, but to my knowledge no successful process has been carried out wherein the anti-oxidants are removed by treatment at room temperature with an oxidizing agent and with controlled acidity or controlled alkalinity with respect to the oil.

According to my process I regulate the acidity or alkalinity of the treating solution, maintaining a value only slightly on the acid or slightly on the alkaline side. I find that at the neutral point (pH of 7.0) it is impossible to effectively treat the oil for the purpose herein set forth, and also if the acidity or alkalinity exceeds a certain predetermined limit which varies only slightly according to the type of oxidizing agent employed, the process becomes less and less effective until a point is reached where substantially no improvement occurs. Accordingly my process consists in treating the oils with a relatively strong oxidizing agent in low concentration with respect to the oil, and within predetermined limits on the acid or alkaline side.

The length of time required for treating these oils is determined by the first measurable increase in refractive index or by a corresponding decrease in iodine number. The method of treatment of an oil comprises treating the oil preferably at room temperature either with an aqueous solution of oxidizing agents such as permanganates, chromates, nitric acid and the like, or with organic oxidizing agents such as peroxides in an alcoholic alkaline solution or an aqueous

acid solution may be employed within the limited alkaline or acid range to be more fully described hereinafter. This process effectively removes the anti-oxidants (such as lecithin and cephalin) which are naturally occurring in these oils. The sludge containing the anti-oxidants and spent reagents may be separated from the refined oil in any suitable manner, such as filtering or centrifuging, depending on the nature of the treating solution. In the case of alcoholic solutions the excess alcohol may be removed by distillation.

I have determined by numerous experiments the optimum of acid or alkaline values and this will be more apparent from a consideration of the accompanying graphs, in which:

Fig. 1 is a general graph showing the relation between the acidity or alkalinity and the time of gelation in hours.

Fig. 2 is a general graph showing the conditions for determining the length of time of treatment.

Fig. 3 is a specific graph showing the effect of regulated quantities of alkali and acid in the presence of a constant amount of potassium permanganate in an aqueous solution.

Fig. 4 is a graph showing the rate of drying of a representative group of untreated soya bean oils.

Fig. 5 is a graph showing the rate of drying of soya bean oils treated with alkali-permanganate reagents.

Fig. 6 is a graph showing the comparative effectiveness of various percentages of acid or alkali on the total drying time of oils treated with various reagents.

Fig. 7 is a graph showing the rate of drying of oils treated with acid-permanganate reagents.

Fig. 8 is a graph showing the rate of drying of oils treated with nitric acid reagents.

Fig. 9 is a graph comparing untreated soya bean oils, treated soya bean oils and raw linseed oil with respect to the time required to come to complete gelation.

The graphs are largely self-explanatory. It will be noted however that the rate of diffusion is greater in the alkali process than in the acid treatment. The rate of diffusion in turn is controlled by the rate of oxidation. The compound formed by the reaction between alkali and the anti-oxidant is less stable than that formed by the acid and anti-oxidant.

From the maxima of the curves, upward in the case of alkali and downward for acid, it will be noted that increasing amounts of acid or alkali exert a repressive effect on the reaction.

Excessive amounts slow down the reaction to substantially zero.

- Since the anti-oxidant is an amino compound (lecithin or cephalin) it forms salts with the acids. These salts of the acid and amino compounds are more stable than the amino compounds and therefore harder to break down or decompose. With this thought in mind it is evident that the alkali will be more effective than the acid treatment. Experiments have shown this to be the case, the maximum acid concentration based on the percent of acid per 100 parts of oil being about two times the maximum alkali concentration, i. e., about two times more acid than alkali is required to obtain the maximum on the acid side than is required on the alkaline side. This relation applies only to the case of a process employing inorganic oxidizing agents in aqueous solution.
- 20 The optimum treating conditions using an inorganic oxidizing agent may be summarized as follows:

*Alkali treatment*

|                            | Per cent |
|----------------------------|----------|
| 25 Alkali (KOH) -----      | 0.025    |
| KMnO <sub>4</sub> -----    | 1.0      |
| Water (not constant) ----- | 1.0-10   |

*Time of treatment.*—½-8 hours.

*Product.*—An oil slightly lighter than the original in color, and which goes to complete gelation in 25 hours.

*Acid treatment*

|                            | Per cent |
|----------------------------|----------|
| 35 HCl -----               | 0.05     |
| KMnO <sub>4</sub> -----    | 1.0      |
| Water (not constant) ----- | 1.0-10   |

*Time of treatment.*—½-8 hours.

*Product.*—An oil slightly lighter than the original in color, which goes to complete gelation in 60 hours.

While the optimum point for alkali treatment is 0.025% it will be noted satisfactory results may be obtained within the range of .013 to .40. The preferred range however is from .013 to .050 as indicated by the upper graph forming part of Fig. 3. Likewise in connection with the acid treatment while optimum results are obtained with .05% acid, valuable results may be obtained between the range of .02 to .50. The preferred range for the acid treatment is from .025 to .050 as indicated by the lower graph forming part of Fig. 3.

While in most of the above graphs soya bean oil was treated, comparable results are obtained using other drying or semi-drying oils such as linseed oil, sun flower oil, perilla oil, rape seed oil and oiticica oil, the variation in the graphs using these other oils being of an order of plus or minus 5% of the values indicated in the graph.

60 In the above graphs the aqueous solution of an inorganic oxidizing agent was employed.

While the optimum point for oxidizing agents is expressed as 1.0%, comparable results can be obtained using the range from 0.5 to 1.5 parts of oxidizing agent by weight per 100 parts of oil.

65 The invention will be further apparent from the following specific examples which are intended as illustrative only and not as in any way limiting the invention:

|                               | Parts by weight |
|-------------------------------|-----------------|
| 70 Soya bean oil -----        | 100             |
| Potassium permanganate -----  | 1               |
| Potassium hydroxide -----     | .025            |
| 75 Water (not constant) ----- | 1.0-10          |

This mixture is agitated mechanically using a stirrer or by blowing filtered air or an inert gas through the material, it being understood that the air or gas employed functions solely as an agitating means and does not in any way enter into the reaction. This mixture is agitated from 1 to 2 hours preferably at substantially room temperature and the decomposed impurities filtered out.

The exact time of treatment depends on how soon the anti-oxidant is destroyed. The complete destruction of anti-oxidants is determined when the refractive index (Fig. 2) first begins to increase. (The correlation between the index of refraction and iodine number was first established by A. M. Waguet and J. C. Brier (Ind. Eng. Chem., p. 40, Jan. 1931).) The resultant oil is much improved in drying properties and has a slightly lighter color. A film of this treated oil when baked one hour at 200° F. proves to be 20 harder than the best refined linseed oil subjected to the same bake.

*Example 2*

|                              | Parts by weight |
|------------------------------|-----------------|
| Perilla oil -----            | 100             |
| Potassium permanganate ----- | 1               |
| Hydrochloric acid -----      | .05             |
| Water (not constant) -----   | 1.0-10          |

Using the above agitation time and temperature 30 as described in Example 1, this process yields an oil slightly lighter in color than the original and possessing the same improved drying properties referred to in Example 1.

*Example 3*

|                            | Parts by weight |
|----------------------------|-----------------|
| Oiticica oil -----         | 100             |
| Sodium dichromate -----    | 1.5             |
| HCl -----                  | 0.3             |
| Water (not constant) ----- | 1.0-10          |

The operating conditions may be as described in Examples 1 and 2 and the final product possesses similar characteristics.

*Example 4*

|                            | Parts by weight |
|----------------------------|-----------------|
| Raw linseed oil -----      | 100             |
| Sodium dichromate -----    | 1.5             |
| Sodium hydroxide -----     | 0.3             |
| Water (not constant) ----- | 1.0-10          |

Same agitation is in the preceding examples which results in an oil with improved drying properties as described in Examples 1 and 2.

While particular oils have been referred to in the preceding examples it will be understood that various other oils may be substituted with similarly improved drying properties in the final product.

I claim:

1. A process for improving the drying quality of raw oils containing naturally occurring anti-oxidants, which comprises removing the anti-oxidants from such oils by treating the oils at substantially room temperature with a relatively strong inorganic oxidizing agent in concentration of .5-1.5 parts of oxidizing agent per 100 parts by weight of the oil, and maintaining the pH value close to the neutral point while avoiding exact neutrality, by treating the oil with a member of the group consisting of alkaline and acidic reagents, the proportions employed in the case of the alkaline reagent falling within the range of .013-.050 part by weight of alkali to 70 100 parts by weight of the oil, and in the case 75

- of the acid falling within the range of .025-.050 part by weight of acid to 100 parts by weight of the oil.
2. A process for improving the drying quality 5 of raw oils containing naturally occurring anti-oxidants, which comprises removing the anti-oxidants from such oils by treating the oils at substantially room temperature with a relatively strong inorganic oxidizing agent in concentra- 10 tion of .5-1.5 parts of oxidizing agent per 100 parts by weight of the oil, and maintaining the pH value close to the neutral point while avoiding exact neutrality by treating the oil with an alkaline reagent, the proportion of the alkaline 15 reagent employed falling within the range of .013-.050 part by weight of alkali to 100 parts by weight of the oil being treated.
3. A process for improving the drying quality of raw oils containing naturally occurring anti-oxidants, which comprises removing the anti-oxidants from such oils by treating the oils at substantially room temperature with a relatively 5 strong inorganic oxidizing agent in concentra- 10 tion of .5-1.5 parts of oxidizing agent per 100 parts by weight of the oil, and maintaining the pH value close to the neutral point while avoiding exact neutrality by treating the oil with an acid, the proportion of the acid employed falling within the range of .020-.050 part by weight of acid to 100 parts by weight of the oil being treated.

THEODORE S. HODGINS. 15